

# United States Patent Office

2,743,232

Patented Apr. 24, 1956

1

2,743,232

## FIBROUS 2-PHOSPHATOETHYL ETHERS OF CELLULOSE AND PROCESS OF MAKING THE SAME

Leon H. Chance, Jane Warren, and John D. Guthrie, New Orleans, La., assignors to the United States of America as represented by the Secretary of Agriculture

No Drawing. Application July 18, 1952,  
Serial No. 299,771

4 Claims. (Cl. 8—120)

(Granted under Title 35, U. S. Code (1952), sec. 266)

A non-exclusive, irrevocable, royalty-free license in the invention herein described, for all governmental purposes, throughout the world, with the power to grant sub-licenses for such purposes, is hereby granted to the Government of the United States of America.

This invention relates to partial ethers of fibrous cellulose in which the fibrous form, and the properties it produces in textiles, i. e., properties such as hand, feel, tensile strength and the like are retained substantially unaltered. The invention provides: fibrous 2-phosphatoethyl partial ethers of cellulose; the salts of such ethers; and a process of reducing the combustibility of fibrous cellulosic materials.

We have discovered that bringing a cellulosic material containing hydroxyl groups into contact with a solution consisting of an alkali metal salt of 2-chloroethylphosphoric acid (2-chloroethyl dihydrogen phosphate) and unreacted alkali metal hydroxide dissolved in water, at a temperature at which reaction takes place results in a conversion of hydroxyl groups of the cellulosic material to 2-phosphatoethyl groups ( $-\text{OCH}_2\text{CH}_2\text{OPO}_3^-$ ), and that little saponification of the chloorethyl phosphate takes place.

According to this invention, fibrous alkali metal salts of 2-phosphatoethyl partial ethers of cellulose are produced by reacting fibrous cellulosic materials containing hydroxyl groups with an aqueous solution of an alkali metal salt of 2-chloroethylphosphoric acid (or other salts of 2-chloroethylphosphoric acid may be used in which the alkali metal will replace the cations of the salt) and an excess of alkali metal hydroxide. The corresponding dibasic acid esters are produced by contacting the fibrous alkali metal salts thus produced with a dilute aqueous strong mineral acid until substantially all of the alkali metal atoms have been replaced by hydrogen atoms.

The combustibility of fibrous cellulosic materials containing hydroxyl groups are reduced by converting the cellulosic materials to the corresponding dibasic acid ethers in the above manner and contacting such ethers with ammonia until substantially one equivalent of ammonia per mole of phosphorus has been neutralized, the acid hydrogens of the dibasic acid esters being replaced with  $\text{NH}_4$  groups.

Substantially any fibrous cellulosic material, which contains hydroxyl groups and which can be mercerized, can be phosphatoethylated by the process of this invention. Suitable cellulosic materials include: cotton fibers, regenerated cotton fibers, aminated cotton fibers, carboxymethylated cotton fibers, paper, and the like materials. The use of cotton fibers is preferred.

The fibrous cellulosic materials can be phosphatoethylated in the form of free fibers, sliver, yarn, or fabric. The use of fabric is preferred.

The alkali metal salt of 2-chloroethylphosphoric acid for use in the invention can be prepared by a variety of known procedures. One method comprises: preparing 2-chloroethylphosphoryl dichloride by the method of Renshaw and Hopkins, J. Am. Chem. Soc. 51, 953—4, hydro-

2

lyzing the dichloride with water and reacting the resultant acid with an alkali metal. The substantially neutral sodium or potassium salts of 2-chloroethylphosphoric acid are particularly suitable.

5 Aqueous solutions of the alkali metal or other salts of 2-chloroethylphosphoric acid and excess or unreacted alkali metal hydroxide suitable for use in the present process can be aqueous solutions of the salt and any alkali metal hydroxide containing from about 8 to 25% by weight unreacted alkali metal hydroxide and from about 5 to 15% by weight of the alkali metal salt of 2-chloroethylphosphoric acid. Aqueous solutions of the sodium salt of the acid containing from about 14 to 20% unreacted sodium hydroxide and from about 10 to 12% of the sodium salt of the acid are preferred.

The fibrous cellulosic material can be reacted with such aqueous solutions in a variety of manners. For example, the cellulosic material can be impregnated with an aqueous solution of 2-chloroethylphosphoric acid, or 20 any soluble salt thereof, followed by an impregnation of the resultant wet fabric with an aqueous solution of an alkali metal hydroxide; using, in each step, solution concentrations and solution pick-ups of such magnitude that the resultant aqueous solution which is finally in contact with the fabric contains organophosphate anions and unreacted alkali metal hydroxide in about the indicated proportions. Alternatively the cellulosic material can be impregnated with a solution consisting of 2-chloroethylphosphoric acid, or a soluble salt thereof, dissolved along 30 with an alkali metal hydroxide in water to make a solution containing about the indicated proportions of unreacted alkali metal hydroxide and the acid. The latter method is preferred.

35 The impregnation of the fibrous cellulosic material can be accomplished by any of the conventional procedures for impregnating such materials with solutions; for example, by the procedures for impregnating such materials with mercerizing solutions. The use of a textile padder in the impregnation step is preferred.

40 The reaction can be conducted at temperatures ranging from about room temperature (i. e., about 20° C.) to temperatures at which the thermal decomposition of the cellulosic material becomes appreciable. Cotton fabric is preferably padded with an aqueous solution containing the organophosphate anions and unreacted alkali metal hydroxide to a pick-up of from about 100 to 150% and heated at from about 80 to 110° C. for from about 5 to 40 minutes, using a shorter time with a higher temperature.

45 The impregnated fibrous cellulosic material can be heated in the conventional textile material heating apparatus such as ovens, hot boxes, steam heated cans and the like. After the desired extent of reaction is completed, the fibrous cellulosic material is preferably washed free of any excess reactants and dried by a conventional textile drying procedure. Washing with water and air drying are preferred.

50 The phosphatoethylation process produces an alkali metal salt of a fibrous 2-phosphatoethyl partial ether of cellulose. These ether products are valuable cation exchange materials. For example, cotton fabrics phosphatoethylated, using a sodium salt of 2-chloroethylphosphoric acid in the presence of unreacted sodium hydroxide, constitute ion exchange fabrics in the sodium cycle of the ion exchange process. By the conventional procedures of ion exchange, such fabrics can be converted to the hydrogen cycle and the hydrogen atoms can be replaced by substantially any cation dissolved in an aqueous medium. In such ethers the phosphorus is bound to the molecules of cellulose by relatively strong bonds. For example, when a phosphatoethylated cotton fabric is subjected to the Number 4 wash test of the American Association of Textile

Chemists and Colorists, it undergoes no reduction in phosphorus content.

Fibrous dibasic 2-phosphatoethyl partial ethers of cellulose are preferably prepared by contacting the alkali metal salts of fibrous 2-phosphatoethyl cellulosic materials with a dilute aqueous solution of a strong inorganic acid. The use of aqueous solutions containing from about 3 to 10% of acids such as hydrochloric or sulfuric acid is preferred. The contact is preferably maintained until substantially all of the alkali metal atoms have been replaced by hydrogen atoms as determined by immersion in standard base and back-titration with standard acid. The resultant dibasic acid ethers are preferably washed free of excess reactants. Water washing is preferred. Such fibrous dibasic acid ethers exhibit a marked resistance to burning when they contain about 2% or more of phosphorus and they constitute valuable cellulosic materials which are capable of reacting with many compounds by the typical reactions of organic monoesters of phosphoric acid. Such fibrous dibasic acid ethers are relatively stable compounds, but when they are dried and stored for several weeks the fiber strength decreases markedly.

The combustibility of fibrous cellulosic materials is preferably reduced by treating the materials in the form of fabrics. The treatment is preferably applied to cotton fabrics. The fabric is preferably phosphatoethylated to a phosphorus content of at least about 0.25%. Much higher phosphorus contents can be used in producing fabrics for many applications although fabrics containing more than about 2.5% phosphorus tend to become stiff and boardy. The resultant alkali metal salts are preferably converted to the dibasic acid form and contacted with an aqueous solution containing from about 2 to 5% of ammonia until substantially one equivalent of ammonia per mole of phosphorus has been neutralized. Alternatively, the acid form of the phosphatoethylated cellulosic materials can be contacted with gaseous ammonia or with a solution containing unreacted ammonia.

Even when cellulosic material contains as little as 0.25% phosphorus, the ammonium salts of such fibrous materials exhibit a reduced combustibility. In addition, when they do burn, they produce a black char which exhibits no afterglow. Since the production of such a char and the lack of afterglow are important characteristics of a flameproofed fabric, the present process can advantageously be used as a supplement to other flameproofing processes to enhance the char and afterglow characteristics of the flameproofed fabric. Ammonium salts of phosphatoethylated fibrous cellulosic materials containing at least about 2% phosphorus will not burn even when materials composed of such fibers are held in a vertical position and lighted at the bottom.

Thus the produced chemically modified textile fibers are modified only in that a plurality of the hydroxyl groups of the cellulose contained in the fibers are converted to  $OCH_2CH_2OPO_3M_2$  groups in which M is hydrogen or  $NH_4$ . The degree of conversion is such that the modified cotton has about 0.25 to 2.5% phosphorus contained in the  $OCH_2CH_2OPO_3M_2$  group.

The following examples are illustrative of the invention.

*Combustibility tests.*—The cloths prepared in the following examples were cut into strips 1 cm. wide and at least 5 cm. long. The strips were held with their surface vertical and their long edge at the indicated angle from the vertical and ignited at the specified point. Whether or not the burning would continue along the strip and the presence or absence of afterglow were observed. Strips of the cloths used in each of the examples, prior to treatment, would burn continuously even when held vertically and ignited at the top.

#### EXAMPLE 1

##### *Phosphatoethylation*

Cotton print cloth was padded with a solution consist-

ing of: 150 parts sodium salt of 2-chloroethylphosphoric acid, 850 parts aqueous 25% sodium hydroxide, and 200 parts water. (Solution pick-up was 136%). The wet cloth was heated at 110° C. for 18 minutes, padded with aqueous 25% sodium hydroxide (pick-up 105%), heated at 10° C. for 30 minutes, washed and dried.

The cloth contained 1.34% phosphorus and 11.1% moisture. After laundering (AATCC 36-45 No. 4 test—using 0.5% soap, 0.2% sodium carbonate, and 0.1% chlorine at 182° F for 45 min.) the cloth contained 1.32% phosphorus and 10.4% moisture.

A sample of the same cloth after boiling for 6 hours in 1% sodium hydroxide solution contained 1.36% phosphorus and 9.0% moisture.

A strip of the cloth held at an angle of 90° from the vertical and lighted at one end burned continuously, but a strip held at 45° from the vertical and lighted at the upper end would not burn continuously. The strips exhibited some afterglow.

#### *Ammonium salt production*

A portion of the cloth converted to the ether sodium salt in the above manner was soaked for 10 minutes in 5% hydrochloric acid, washed free of acid with water, soaked for 10 minutes in 5% ammonium hydroxide, washed with water, and dried. It now contained 1.39% phosphorus, 0.69% nitrogen, and 8.0% moisture.

A strip of the cloth held vertically and lighted at the lower end would burn continuously, but one held at an angle of 165° and lighted at the lower end would not burn continuously. The strip exhibited no afterglow.

#### EXAMPLE 2

##### *Separate application of 2-chloroethylphosphoric acid*

Cotton print cloth was impregnated with aqueous 18% sodium hydroxide, allowed to stand for 15 minutes, and then impregnated with a solution consisting of water and a neutral sodium salt of 2-chloroethylphosphate containing about 33% organophosphate anions. The wet cloth was heated at 110° C. for 15 minutes, cooled, re-impregnated with the acid salt, heated at 110° C. for 35 minutes, washed, and dried.

The cloth had a cation exchange capacity of 1.5 milliequivalents per gram and contained 2.68% phosphorus.

After material prepared above was acidified and converted to the ammonium salt by the procedure described in Example 1, a strip of the cloth held vertically and lighted at the bottom would not burn continuously. No afterglow was observed.

#### EXAMPLE 3

##### *Reaction at room temperature*

Cotton print cloth was impregnated with aqueous 18% sodium hydroxide, twice impregnated with a solution consisting of water and a neutral sodium salt of 2-chloroethylphosphoric acid containing about 33% organophosphate anions and allowed to stand for 6.5 days at room temperature.

The cloth exhibited a cation exchange capacity of 1.7 milliequivalents per gram.

A sample of the cloth was acidified and converted to the ammonium salt by the procedure of Example 1. A strip of the resultant cloth held vertically and lighted at the bottom would not burn continuously. No afterglow was observed.

#### EXAMPLE 4

##### *Curing times and temperatures in relation to combined phosphorus*

Cotton print cloth was impregnated with a solution consisting of water, sodium hydroxide and a sodium salt of 2-chloroethylphosphoric acid containing 10% unreacted sodium hydroxide and 20% organophosphate anions (132% pick-up). Portions of the wet cloth were heated

in a forced draft oven for the indicated times and temperatures.

The cation exchange capacities and the phosphorus content of the samples of the cloth are reported in the following table.

| Curing time | Cation-exchange capacity in milliequiv. per g. (dry basis) |        |         |         | Phosphorus content in percent (dry basis) |        |         |         |
|-------------|------------------------------------------------------------|--------|---------|---------|-------------------------------------------|--------|---------|---------|
|             | 80° C.                                                     | 90° C. | 100° C. | 110° C. | 80° C.                                    | 90° C. | 100° C. | 110° C. |
| 5 min.      | 0.15                                                       | 0.10   | 0.54    | 0.48    | 0.23                                      | 0.24   | 1.10    | 1.07    |
| 10 min.     | 0.42                                                       | 0.55   | 0.57    | 0.56    | 0.81                                      | 1.06   | 1.15    | 1.12    |
| 20 min.     | 0.46                                                       | 0.62   | 0.59    | 0.58    | 0.96                                      | 1.26   | 1.18    | 1.17    |
| 40 min.     | 0.45                                                       | 0.68   | 0.60    | 0.59    | 1.02                                      | 1.29   | 1.31    | 1.17    |

### EXAMPLE 5

#### Unreacted alkali metal hydroxide concentration in relation to combined phosphorus

Samples of cotton print cloth were padded with solutions of sodium salt of 2-chloroethylphosphoric acid, sodium hydroxide and water containing 10% organophosphate anions and the indicated amounts of unreacted sodium hydroxide (130% average pick-up). The wet cloths were heated for 20 minutes at 100° C., washed and air dried.

The cation exchange capacities and phosphorus content of the so treated cloths are expressed in the following table.

| Percent Unreacted NaOH | Cation-exchange capacity, milliequivalents per g. (dry basis) | Percent Phosphorus (dry basis) |
|------------------------|---------------------------------------------------------------|--------------------------------|
| 8                      | 0.52                                                          | 0.98                           |
| 12                     | 0.70                                                          | 1.18                           |
| 14                     | 0.78                                                          | 1.28                           |
| 16                     | 0.81                                                          | 1.32                           |
| 18                     | 0.79                                                          | 1.36                           |
| 20                     | 0.75                                                          | 1.31                           |
| 22                     | 0.68                                                          | 1.12                           |

### EXAMPLE 6

#### Chloroethyl phosphate acid anion concentration in relation to combined phosphorus

Samples of cotton print cloth were padded with a solution of the sodium salt of 2-chloroethylphosphoric acid, sodium hydroxide and water containing 16% unreacted sodium hydroxide and the indicated amounts of organophosphate anions (130% average pick-up). The wet cloths were heated 20 minutes at 100° C., washed and air dried.

The cation exchange capacities and the phosphorus content of the so treated cloths are indicated in the following table.

| Percent 2-chloroethyl phosphoric acid anions | Cation-exchange capacity, milliequiv. per g. | Percent Phosphorus |
|----------------------------------------------|----------------------------------------------|--------------------|
| 5                                            | 0.43                                         | 0.72               |
| 7                                            | 0.59                                         | 0.95               |
| 10                                           | 0.78                                         | 1.30               |
| 12                                           | 0.79                                         | 1.34               |
| 15                                           | 0.67                                         | 1.13               |
| 18                                           | 0.54                                         | 0.96               |

### EXAMPLE 7

#### Repeated phosphatoethylation

Cotton print cloth was padded with a solution of sodi-

70

2828-2834, Dec. 1949.

um salt of 2-chloroethylphosphoric acid, sodium hydroxide and water, containing 16% unreacted sodium hydroxide and 10% organophosphate anions (130% pick-up), heated for 20 minutes at 100° C., washed and dried. The resultant cloth had a cation exchange capacity of 0.80 milliequivalents per g. and a phosphorus content of 1.34%.

The cloth was re-treated in the above manner. It then had a cation exchange capacity of 1.5 milliequivalents per g. and a phosphorus content of 2.4%.

The re-treated cloth was converted to the ammonium salt by the process of Example 1. A strip of the so treated cloth held vertically and lighted at the bottom would not support combustion. No afterglow was observed.

We claim:

1. A process comprising impregnating a cotton fabric with an aqueous solution of about 5 to 15% by weight of a sodium salt of 2-chloroethylphosphoric acid and about 14 to 20% by weight of sodium hydroxide, and heating the wet fabric at about 80 to 110° C. for about 5 to 40 minutes, using a shorter time with a higher temperature to produce a modified cotton having about 0.25 to 2.5% phosphorus by weight.

2. A process comprising impregnating a cotton fabric with an aqueous solution of about 5 to 15% by weight of a sodium salt of 2-chloroethylphosphoric acid and about 14 to 20% by weight of sodium hydroxide, heating the wet fabric at about 80 to 110° C. for about 5 to 40 minutes, using a shorter time with a higher temperature to produce a modified cotton having about 0.25 to 2.5% phosphorus by weight.

3. A process comprising impregnating a cotton fabric with an aqueous solution of about 5 to 15% by weight of a sodium salt of 2-chloroethylphosphoric acid and about 14 to 20% by weight of sodium hydroxide, heating the wet fabric at about 80 to 110° C. for about 5 to 40 minutes, using a shorter time with a higher temperature to produce a modified cotton having about 0.25 to 2.5% phosphorus by weight.

4. A process comprising impregnating a cotton fabric with an aqueous solution of about 5 to 15% by weight of a sodium salt of 2-chloroethylphosphoric acid and about 14 to 20% by weight of sodium hydroxide, heating the wet fabric at about 80 to 110° C. for about 5 to 40 minutes, using a shorter time with a higher temperature to produce a modified cotton having about 0.25 to 2.5% phosphorus by weight.

5. A process comprising impregnating a cotton fabric with an aqueous solution of about 5 to 15% by weight of a sodium salt of 2-chloroethylphosphoric acid and about 14 to 20% by weight of sodium hydroxide, heating the wet fabric at about 80 to 110° C. for about 5 to 40 minutes, using a shorter time with a higher temperature to produce a modified cotton having about 0.25 to 2.5% phosphorus by weight.

6. A process comprising impregnating a cotton fabric with an aqueous solution of about 5 to 15% by weight of a sodium salt of 2-chloroethylphosphoric acid and about 14 to 20% by weight of sodium hydroxide, heating the wet fabric at about 80 to 110° C. for about 5 to 40 minutes, using a shorter time with a higher temperature to produce a modified cotton having about 0.25 to 2.5% phosphorus by weight.

7. A process comprising impregnating a cotton fabric with an aqueous solution of about 5 to 15% by weight of a sodium salt of 2-chloroethylphosphoric acid and about 14 to 20% by weight of sodium hydroxide, heating the wet fabric at about 80 to 110° C. for about 5 to 40 minutes, using a shorter time with a higher temperature to produce a modified cotton having about 0.25 to 2.5% phosphorus by weight.

8. A process comprising impregnating a cotton fabric with an aqueous solution of about 5 to 15% by weight of a sodium salt of 2-chloroethylphosphoric acid and about 14 to 20% by weight of sodium hydroxide, heating the wet fabric at about 80 to 110° C. for about 5 to 40 minutes, using a shorter time with a higher temperature to produce a modified cotton having about 0.25 to 2.5% phosphorus by weight.

9. A process comprising impregnating a cotton fabric with an aqueous solution of about 5 to 15% by weight of a sodium salt of 2-chloroethylphosphoric acid and about 14 to 20% by weight of sodium hydroxide, heating the wet fabric at about 80 to 110° C. for about 5 to 40 minutes, using a shorter time with a higher temperature to produce a modified cotton having about 0.25 to 2.5% phosphorus by weight.

#### References Cited in the file of this patent

##### UNITED STATES PATENTS

2,256,380 Dickey et al. Sept. 16, 1941  
2,265,585 Urbain et al. Dec. 9, 1941

##### FOREIGN PATENTS

837,592 France Feb. 14, 1939  
343,873 Great Britain Feb. 16, 1931

##### OTHER REFERENCES

Reid et al.: Ind. and Eng. Chemistry, vol. 41, #12, pp. 2828-2834, Dec. 1949.